



US007763744B2

(12) **United States Patent**  
Tynik et al.

(10) Patent No.: US 7,763,744 B2  
(45) Date of Patent: Jul. 27, 2010

- (54) **MOLYBDENUM DIALKYLDITHIOCARBAMATE COMPOSITIONS AND LUBRICATING COMPOSITIONS CONTAINING THE SAME**

(75) Inventors: **Robert J. Tynik**, Norwalk, CT (US);  
**Steven G. Donnelly**, Bethel, CT (US);  
**Thomas J. Karol**, Holualoa, HI (US)

(73) Assignee: **R.T. Vanderbilt Company, Inc.**,  
Norwalk, CT (US)

(\*) Notice: Subject to any disclaimer, the term of the patent is extended or adjusted under U.S.C. 154(b) by 1005 days.

(21) Appl. No.: **11/363,896**

(21) Appl. No.: 11/363,896

(22) Filed: **Feb. 28, 2006**

(65) **Prior Publication Data**

US 2006/0199745 A1 Sep. 7, 2006

### Related U.S. Application Data

- (60) Provisional application No. 60/657,610, filed on Mar. 1, 2005.

(51) **Int. Cl.**  
*C07F 11/00* (2006.01)  
*C10M 159/18* (2006.01)

(52) **U.S. Cl.** ..... **556/63**; 556/38; 556/50;  
508/230; 508/363

(58) **Field of Classification Search** ..... 508/230,  
508/363; 556/50, 63

(56) **References Cited**

## U.S. PATENT DOCUMENTS

- 3,356,702 A 12/1967 Farmer et al.  
 3,509,051 A 4/1970 Farmer et al.

|           |   |         |                |       |            |
|-----------|---|---------|----------------|-------|------------|
| 4,098,705 | A | 7/1978  | Sakurai et al. | ..... | 252/33.6   |
| 4,178,258 | A | 12/1979 | Papay et al.   | ..... | 252/32.7 E |
| 4,529,526 | A | 7/1985  | Inoue et al.   | ..... | 252/32.7   |

(Continued)

## FOREIGN PATENT DOCUMENTS

JP 62081396 A 4/1987

#### OTHER PUBLICATIONS

Tomah Products Technical Data Sheet DA 1618, May 2, 1996, 337  
Vincent Street Milton, WI 53563, pp. 1-4.\*

*Primary Examiner*—Ellen M McAvoy

*Assistant Examiner*—Vishal Vasisth

(74) *Attorney, Agent, or Firm*—Norris, McLaughlin & Marcus

## ABSTRACT

The invention relates to a novel asymmetrical, secondary dialkylamine-based molybdenum dithiocarbamate with improved friction reducing performance, viscosity and solubility, and lubricating compositions containing the same. The compounds are produced from asymmetrical dialkylamine of the formula R1-NH—R2 where R1 and R2 are different, and are independently selected from alkyl groups C3 to C19. In a preferred embodiment, R3 and R4 are different and are independently selected from alkyl groups C3 to C19. The molybdenum dithiocarbonates can be represented by the following formula:



$$\begin{aligned}v &= 1-2; \\w &= 1-2; \\x + y &= 2-5; \\z &= 1-2\end{aligned}$$

**8 Claims, 2 Drawing Sheets**



ASTM D5707-2004: 50M - 80°C: 1H: 1mm Stroke: Ball-on-Disc

# US 7,763,744 B2

Page 2

---

## U.S. PATENT DOCUMENTS

|               |         |                         |          |                 |         |                        |         |
|---------------|---------|-------------------------|----------|-----------------|---------|------------------------|---------|
| 4,692,256 A * | 9/1987  | Umemura et al. ....     | 508/362  | 5,840,672 A     | 11/1998 | Gatto .....            | 508/334 |
| 4,705,766 A   | 11/1987 | Howell et al. ....      | 502/167  | 5,916,851 A     | 6/1999  | Hosonuma et al.        |         |
| 4,846,983 A   | 7/1989  | Ward, Jr. ....          | 252/33.6 | 5,939,364 A     | 8/1999  | Polizzotti et al. .... | 508/363 |
| 5,281,347 A   | 1/1994  | Igarashi et al. ....    | 252/42.7 | 5,994,277 A     | 11/1999 | Ritchie et al. ....    | 508/365 |
| 5,356,547 A   | 10/1994 | Arai et al.             |          | 6,074,993 A     | 6/2000  | Waddoups et al. ....   | 508/364 |
| 5,445,749 A * | 8/1995  | Hong .....              | 508/443  | 6,103,674 A     | 8/2000  | Nalesnik et al. ....   | 508/334 |
| 5,494,608 A   | 2/1996  | Kamakura et al. ....    | 252/42.7 | 6,245,725 B1    | 6/2001  | Tanaka et al. ....     | 508/365 |
| 5,605,880 A   | 2/1997  | Arai et al. ....        | 508/379  | 6,268,316 B1    | 7/2001  | Tanaka et al. ....     | 508/291 |
| 5,627,146 A   | 5/1997  | Tanaka et al. ....      | 508/363  | 6,300,291 B1    | 10/2001 | Hartley et al. ....    | 508/363 |
| 5,696,065 A   | 12/1997 | Tanaka et al.           |          | 6,329,328 B1    | 12/2001 | Koganei et al. ....    | 508/365 |
| 5,744,430 A   | 4/1998  | Inoue et al. ....       | 508/295  | 6,444,624 B1    | 9/2002  | Walker et al. ....     | 508/363 |
| 5,814,587 A   | 9/1998  | Vrahopoulou et al. .... | 508/363  | 2003/0224951 A1 | 12/2003 | McConnachie et al.     |         |

\* cited by examiner



FIG. 1



FIG. 2

## 1

**MOLYBDENUM  
DIALKYLDITHIOCARBAMATE  
COMPOSITIONS AND LUBRICATING  
COMPOSITIONS CONTAINING THE SAME**

This application is a Continuation of Ser. No. 60/657,610, filed Mar. 1, 2005.

BACKGROUND OF THE INVENTION

1. Field of the Invention

The invention relates to novel asymmetric molybdenum dialkyldithiocarbamates, prepared from asymmetric dialkylamines, which are useful as additives in lubricating compositions.

2. Discussion of the Prior Art

Molybdenum dithiocarbamates are well-known additives for lubrication formulation. Molybdenum dialkyldithiocarbamates prepared from symmetrical dialkylamines and mixtures of symmetrical dialkylamines are currently used as additives in lubricating oils (as well as mixtures thereof) for imparting antifriction properties. While these compositions are quite effective, there is a desire for compounds that will offer improvements or provide even greater lubricating properties. Also, in certain lubricating oil compositions, prior art molybdenum dialkyldithiocarbamates do not have the desired solubility, especially at lower temperatures, so that the compound separates from the lubricating composition, resulting in the formation of a haze, cloud or precipitate in the lubricating composition, thus reducing its effectiveness.

Therefore, there is also a desire for molybdenum dialkyldithiocarbamates with improved solubility in lubricating compositions. In addition, current molybdenum dithiocarbamates (DTCs) require the addition of substantial amounts of diluent oil to lower the viscosity of the additive to acceptable levels for handling. This reduces the activity of the additive by dilution. Therefore, additives that require less diluent oil to afford a readily pourable product are advantageous. Molybdenum dithiocarbamates can be rendered according to the following formula (1):



$v = 1-2$ ;  
 $w = 1-2$ ;  
 $x + y = 2-5$ ;  
 $z = 1-2$

A particular type of asymmetric molybdenum dithiocarbamate (Mo DTC) is known, in which the R1 and R2 group on one side of the molybdenum groups differ from the R3 and R4 groups on the other side. However, these compounds are believed to be formed by a mixture of two different symmetric dialkylamines, HNR1R2 and HNR3R4, where R1=R2 and R3=R4, and R1 is not the same as R3. For example, U.S. Pat. No. 5,627,146 to Tanaka, et al. describes lubricating oil compositions that contain specifically  $\text{C}_8$  dithiocarbamyl and  $\text{C}_{13}$  dithiocarbamyl ligands to produce an asymmetric type molybdenum dithiocarbamate as an essential component thereof.

A further Tanaka patent U.S. Pat. No. 6,245,725 does speak generally of asymmetric Mo DTC compounds wherein R1, R2, R3 and R4 must merely have one dissimilar alkyl to establish asymmetry, and also states generally that compounds may be formed from a secondary amine having dif-

## 2

ferent hydrocarbon groups. Furthermore, the patent suggests that asymmetric Mo DTC's should be blended with symmetric Mo DTC's in order to achieve good performance. However, such a compound would have been an impossibility at the time of Tanaka's teaching, since such asymmetric dialkylamines did not exist at that time. Only recently have such amines become available, such as (2-ethylhexyl) tridecylamine from Nova Molecular Technologies, Inc. of Janesville, Wis., USA; and isodecyloxypropyl-isopropylamine and alkoxypropyl-isopropyl (alkyl=C12 to C15), from Tomah Products, Inc. of Milton, Wis., USA.

Accordingly, it is seen that the only working example in the '725 patent is the same C8/C 13 Mo DTC as taught by the Tanaka '146 patent. There is no suggestion that such asymmetric dialkylamines were available at that time, and the patent merely relies on two different secondary amines, one C8 and the other C13. Since it would not have been possible to even formulate such compounds at that time, it could also not have been foreseen that, not only are such compounds (based on asymmetric dialkylamines) possible, but that they surprisingly provide even greater friction performance than either symmetric Mo DTCs or the asymmetric Mo DTC taught by Tanaka which is formed from two different symmetric dialkyl amines.

Equally surprising is the discovery that the novel asymmetric compositions have lower viscosity than the composition taught by Tanaka. As less diluent oil is needed for handling, the result is that a lubricating composition, such as a base oil composition, can comprise a greater amount of molybdenum than can the prior art compounds. Thus, the inventive compositions allow for a lubricating composition having up to 12-15% weight percent molybdenum, compared to only about 7.5% maximum when using a symmetric Mo DTC.

SUMMARY OF THE INVENTION

In order to overcome the shortcomings of the existing molybdenum dithiocarbamate compounds in lubricating compositions, applicants have discovered novel asymmetric Mo DTCs formed from asymmetrical dialkyl secondary amines. Such compounds are formed by dialkyl amines of the general formula HNR1R2, where R1 and R2 are dissimilar. Examples of such amines include (2-ethylhexyl) tridecylamine, isodecyloxypropyl-isopropylamine and alkoxypropyl-isopropyl (alkyl=C12 to C15, i.e. presumably derived from a mixture of fatty alcohols containing C12 to C15 straight-chain alcohols). When Mo DTCs are formed by such amines according to known methods, the result is a Mo DTC according to formula 1 in which R1 does not equal R2. If a single asymmetric amine is the source, then R3 and R4 would be the same as R1 and R2, respectively. However, if the amine source also includes a second asymmetric amine, then it is also possible that at least one of R3 or R4 differs from at least one of R1 and R2. Likewise, an amine source based on a mixture of asymmetric and symmetric amines could give a Mo DTC in which R3 and R4 were the same, but different from at least one of R1 and R2.

The invention also relates to lubricating compositions containing an effective amount of the novel asymmetric molybdenum dithiocarbamates. The novel and improved lubricant additives have improved friction reduction properties, better solubility, and allow for a higher molybdenum content afforded by a lower diluent requirement for utility. In particular, the invention relates to novel molybdenum dialkyldithiocarbamates prepared from asymmetric dialkylamines, mixtures of asymmetric dialkylamines or mixtures of asymmetric and symmetric dialkylamines, mixtures of these molybde-

num dialkyldithiocarbamates with other molybdenum dialkyldithiocarbamates, lubricating compositions containing said compounds and mixtures; as well as a method for improving the solubility of a MoDTC in a lubricating composition, a method for preparing a MoDTC having improved viscosity, a method for preparing a lubricating composition with increased friction reduction, and a method for preparing a MoDTC having increased molybdenum content.

It has now been discovered that a novel class of molybdenum dialkyldithiocarbamates imparts improved antifriction properties to lubricants, has generally improved solubility in lubricating compositions and has lower additive viscosities. The lower intrinsic viscosities allow the use of less diluent oil providing higher molybdenum-content additives. In addition, the admixture of these novel compounds with other molybdenum dialkyldithiocarbamates enhances the solubility of the other molybdenum dialkyldithiocarbamates. The novel molybdenum dialkyldithiocarbamates are prepared from asymmetric dialkylamines or mixtures of asymmetric dialkylamines according to a method known in the prior art. However, the inventive compounds and resulting lubricating compositions were not possible in view of the prior art, and their surprising improved properties could not have been foreseen.

#### BRIEF DESCRIPTION OF THE DRAWINGS

FIG. 1 shows a graph comparing friction properties of the inventive compound compared to prior art compounds.

FIG. 2 shows a graph comparing viscosity properties of the inventive compound compared to prior art compounds.

#### DETAILED DESCRIPTION OF THE INVENTION

Molybdenum dithiocarbamates are complexes of an inorganic core with dithiocarbamic acid. Bridged or single molybdenum ("mono-nuclear") cores have been theorized. Additionally, coordination spaces on the molybdenum core may be filled with free amine or other coordinating moieties. This invention relates to the novel compounds formed by utilization of the relatively new asymmetrical dialkyl amine (with different alkyl groups) and the unexpected improvements achieved by this new technology.

The novel molybdenum dialkyldithiocarbamates are prepared by any of a number of methods known to those skilled in the art, such as, but not limited to, the reaction of molybdenum trioxide, water, carbon disulfide and one or more asymmetric dialkylamines HNR1R2, where R1 and R2 are dissimilar. R1 and R2 are independently selected from branched or straight chain groups containing 3 to 19 carbon atoms and preferable C8 to C13 and branched chain to achieve higher solubility effects. Mixtures of asymmetric and symmetric dialkylamines can also be used. This would be expected to form new technology as we have seen that the ligands "scramble". Molybdenum complexes are typically theorized as having 2 dithiocarbamyl ligands. Therefore, the molecule formed by utilization of symmetric and asymmetric dialkyl amine would afford a novel molecule with one of each dithiocarbamyl ligand on the complex. Therefore, the novel invention would be produced in substantial amounts even from small amount of the asymmetrical dialkylamine utilized in the molybdenum dithiocarbamate synthesis.

Applicants have now discovered that Mo DTCs, preferably manufactured from asymmetric dialkylamine starting groups, provide surprisingly superior friction reduction when compared to the prior art compounds. In particular, symmetric Mo DTCs in which R1 is different from R2, and R3 is different from R4, provide superior performance compared to

compounds where R1=R2 and R3=R4. In this respect, applicant's compounds are not necessarily asymmetrical, in that R1 and R3 may both be the same and R2 and R4 may be the same, where R1 does not equal R2. It is also contemplated that compounds formed from two different asymmetric diamines would similarly have superior friction properties. Accordingly, the invention comprises molybdenum dialkyl dithiocarbamates formed by at least one asymmetric dialkylamine. The inventive compounds are such that at least R1 does not equal R2; and preferably, further wherein R3 does not equal R4. It is also noted that excellent results are obtained, in particular as to friction reduction, in the absence of an asymmetric Mo DTC as required by Tanaka '725

The groups, which may form R1 through R4, are well known in the art, for example as set forth in the Tanaka patents referenced above. In addition, the groups that may form R1 through R4 may also contain heteroatoms, such as oxygen and sulfur.

The improved antioxidant, antiwear compositions of the invention may be incorporated in the lubricating compositions by known methods in an amount effective to produce the desired oxidation inhibiting characteristics, for example as 20 0.01 to 15 percent by weight based on the total weight of the lubricating composition. In one embodiment of the invention, the amount may range from about 0.01 to 5.0 percent by weight based on the total weight of the lubricating composition. In another embodiment of the invention, the amount range is about 0.1 to 3.0 percent of the additive based on the total weight of the lubricating composition. The compositions 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9

11. Rust inhibitors  
12. Copper corrosion inhibitors

1. Borated and/or Non-Borated Dispersants

Non-borated ashless dispersants may be incorporated within the final fluid composition in an amount comprising up to 10 weight percent on an oil-free basis. Many types of ashless dispersants listed below are known in the art. Borated ashless dispersants may also be included.

(A) "Carboxylic dispersants" are reaction products of carboxylic acylating agents (acids, anhydrides, esters, etc.) containing at least about 34 and preferably at least about 54 carbon atoms reacted with nitrogen-containing compounds (such as amines), organic hydroxy compounds (such aliphatic compounds including monohydric and polyhydric alcohols, or aromatic compounds including phenols and naphthols), and/or basic inorganic materials. These reaction products include imide, amide and ester reaction products of carboxylic acylating agents. Examples of these materials include succinimide dispersants and carboxylic ester dispersants. The carboxylic acylating agents include alkyl succinic acids and anhydrides wherein the alkyl group is a polybutyl moiety, fatty acids, isoaliphatic acids (e.g., 8-methyloctadecanoic acid), dimer acids, addition dicarboxylic acids, addition (4+2 and 2+2) products of an unsaturated fatty acid with an unsaturated carboxylic reagent), trimer acids, addition tricarboxylic acids (e.g., Empol® 1040, Hystrene® 5460 and Unidyme® 60), and hydrocarbyl substituted carboxylic acylating agents (from olefins and/or polyalkenes). In one preferred embodiment, the carboxylic acylating agent is a fatty acid. Fatty acids generally contain from about 8 up to about 30, or from about 12 up to about 24 carbon atoms. Carboxylic acylating agents are taught in U.S. Pat. Nos. 2,444,328, 3,219, 666 and 4,234,435, which are incorporated herein by reference. The amine may be a mono- or polyamine. The monoamines generally have at least one hydrocarbyl group containing 1 to about 24 carbon atoms, with from 1 to about 12 carbon atoms. Examples of monoamines include fatty (C8-C30) amines, primary ether amines (SURFAM® amines), tertiary-aliphatic primary amines ("Primene"), hydroxyamines (primary, secondary or tertiary alkanol amines), ether N-(hydroxyhydrocarbyl)amines, and hydroxyhydrocarbyl amines ("Ethomeens" and "Propomeens"). The polyamines include alkoxyLATED diamines ("Ethoduomeens"), fatty diamines ("Duomeens"), alkylenepolyamines (ethylenopolyamines), hydroxy-containing polyamines, polyoxyalkylene polyamines (such as JEFFAMINES), condensed polyamines (a condensation reaction between at least one hydroxy compound with at least one polyamine reactant containing at least one primary or secondary amino group), and heterocyclic polyamines. Useful amines include those disclosed in U.S. Pat. Nos. 4,234,435 and 5,230,714 that are incorporated herein by reference. Examples of these "carboxylic dispersants" are described in British Patent 1,306,529 and in U.S. Pat. Nos. 3,219,666, 3,316,177, 3,340,281, 3,351,552, 3,381, 022, 3,433,744, 3,444,170, 3,467,668, 3,501,405, 3,542,680, 3,576,743, 3,632,511, 4,234,435, and Re 26,433, which are incorporated herein by reference for disclosure of dispersants.

(B) "Amine dispersants" are reaction products of relatively high molecular weight aliphatic or alicyclic halides and amines, preferably polyalkylene polyamines. Examples thereof are described, for example, in U.S. Pat. Nos. 3,275, 554, 3,438,757, 3,454,555, and 3,565,804, which are incorporated herein by reference for disclosure of dispersants.

(C) "Mannich dispersants" are the reaction products of alkyl phenols in which the alkyl group contains at least about

30 carbon atoms with aldehydes (especially formaldehyde) and amines (especially polyalkylene polyamines). The materials described in U.S. Pat. Nos. 3,036,003, 3,236,770, 3,414, 347, 3,448,047, 346,172, 3,539,633, 3,586,629, 3,591,598, 3,634,515, 3,725,480, and 3,726,882 are incorporated herein by reference for disclosure of dispersants.

(D) Post-treated dispersants are obtained by reacting carboxylic, amine or Mannich dispersants with reagents such as urea, thiourea, carbon disulfide, aldehydes, ketones, carboxylic acids, hydrocarbon-substituted succinic anhydrides, nitriles, epoxides, boron compounds, phosphorus compounds or the like. U.S. Pat. Nos. 3,200,107, 3,282,955, 3,367,943, 3,513,093, 3,639,242, 3,649,659, 3,442,808, 3,455,832, 3,579,450, 3,600,372, 3,702,757, and 3,708,422 are incorporated herein by reference for disclosure of dispersants.

(E) Polymeric dispersants are interpolymers of oil-solubilizing monomers such as decyl methacrylate, vinyl decyl ether and high molecular weight olefins with monomers containing polar substituents, e.g., aminoalkyl acrylates or acrylamides and poly-(oxyethylene)-substituted acrylates. Polymer dispersants are disclosed in U.S. Pat. Nos. 3,329,658, 3,449,250, 3,519,656, 3,666,730, 3,687,849, and 3,702,300, which are incorporated herein by reference for disclosure of dispersants and ashless dispersants. Borated dispersants are described in U.S. Pat. Nos. 3,087,936 and 3,254,025, which are incorporated herein by reference for disclosure of borated dispersants.

Also included, as possible dispersant additives are those disclosed in U.S. Pat. Nos. 5,198,133 and 4,857,214, which are incorporated herein by reference. The dispersants of these 30 patents compare the reaction products of an alkenyl succinimide or succinimide ashless dispersant with a phosphorus ester or with an inorganic phosphorus-containing acid or anhydride and a boron compound.

2. Additional Antioxidant Compounds

Other antioxidant may be used in the compositions of the present invention, if desired. Typical antioxidants include hindered phenolic antioxidants, secondary aromatic amine antioxidants, sulfurized phenolic antioxidants, oil-soluble copper compounds, phosphorus-containing antioxidants, organic sulfides, disulfides and polysulfides and the like.

Illustrative sterically hindered phenolic antioxidants include orthoalkylated phenolic compounds such as 2,6-di-tert-butylphenol, 4-methyl-2,6-di-tert-butylphenol, 2,4,6-tri-tert-butylphenol, 2-tert-butylphenol, 2,6-disopropylphenol, 2-methyl-6-tert-butylphenol, 2,4-dimethyl-6-tert-butylphenol, 4-(N,N-dimethylaminomethyl)-2,8-di-tert-butylphenol, 4-ethyl-2,6-di-tert-butylphenol, 2-methyl-6-styrylphenol, 2,6-distyryl-4-nonylphenol, and their analogs and homologs. Mixtures of two or more such mononuclear phenolic compounds are also suitable.

Other preferred phenol antioxidants for use in the compositions of this invention are methylene-bridged alkylphenols, and these can be used singly or in combinations with each other, or in combinations with sterically hindered un-bridged phenolic compounds. Illustrative methylene-bridged compounds include 4,4'-methylenebis(6-tert-butyl o-cresol), 4,4'-methylenebis(2-tert-amyl-o-cresol), 2,2'-methylenebis(4-methyl-6-tert-butylphenol), 4,4'-methylenebis(2,6-di-tert-butylphenol) and similar compounds. Particularly preferred are mixtures of methylene-bridged alkylphenols such as are described in U.S. Pat. No. 3,211,652, which is incorporated herein by reference. Amine antioxidants, especially oil-soluble aromatic secondary amines may also be used in the 55 compositions of this invention. Although aromatic secondary monoamines are preferred, aromatic secondary polyamines are also suitable. Illustrative aromatic secondary monoam-

ines include diphenylamine, alkyl diphenylamines containing 1 or 2 alkyl substituents each having up to about 16 carbon atoms, phenyl-.beta.-naphthylamine, phenyl-p-naphthylamine, alkyl- or aralkyl-substituted phenyl-.beta.-naphthylamine containing one or two alkyl or aralkyl groups each having up to about 16 carbon atoms, alkyl- or aralkyl-substituted phenyl-p-naphthylamine containing one or two alkyl or aralkyl groups each having up to about 16 carbon atoms, and similar compounds.

A preferred type of aromatic amine antioxidant is an alkylated diphenylamine of the general formula:



where  $R_1$  is an alkyl group (preferably a branched alkyl group) having 8 to 12 carbon atoms, (more preferably 8 or 9 carbon atoms) and  $R_2$  is a hydrogen atom or an alkyl group (preferably a branched alkyl group) having 8 to 12 carbon atoms, (more preferably 8 or 9 carbon atoms). Most preferably,  $R_1$  and  $R_2$  are the same. One such preferred compound is available commercially as Naugalube® 438L, a material which is understood to be predominately a 4,4'-dinoxyldiphenylamine (i.e., bis(4-nonylphenyl)(amine)) in which the nonyl groups are branched.

Another useful type of antioxidant for preferred inclusion in the compositions of the invention are one or more liquid, partially sulfurized phenolic compounds such as are prepared by reacting sulfur monochloride with a liquid mixture of phenols--at least about 50 weight percent of which mixture of phenols is composed of one or more reactive, hindered phenols--in proportions to provide from about 0.3 to about 0.7 gram atoms of sulfur monochloride per mole of reactive, hindered phenol so as to produce a liquid product. Typical phenol mixtures useful in making such liquid product compositions include a mixture containing by weight about 75% of 2,6-di-tert-butylphenol, about 10% of 2-tert-butylphenol, about 13% of 2,4,6-tri-tert-butylphenol, and about 2% of 2,4-di-tert-butylphenol. The reaction is exothermic and thus is preferably kept within the range of about 15.degree. C. to about 70.degree. C., most preferably between about 40.degree. C. to about 60.degree. C.

Another useful type of antioxidant are 2,2,4-trimethyl-1,2-dihydroquinoline (TMDQ) polymers and homologs containing aromatized terminal units such as those described in U.S. Pat. No. 6,235,686, which is hereby incorporated by reference.

Mixtures of different antioxidants may also be used. One suitable mixture is comprised of a combination of: (i) an oil-soluble mixture of at least three different sterically hindered tertiary butylated monohydric phenols, which is in the liquid state at 25.degree. C.; (ii) an oil-soluble mixture of at least three different sterically-hindered, tertiary butylated methylene-bridged polyphenols; and (iii) at least one bis(4-alkylphenyl) amine wherein the alkyl group is a branched alkyl group having 8 to 12 carbon atoms, the proportions of (i), (ii) and (iii) on a weight basis falling in the range of 3.5 to 5.0 parts of component (i) and 0.9 to 1.2 parts of component (ii) per part by weight of component (iii), as disclosed in U.S. Pat. No. 5,328,619, which is incorporated herein by reference.

Other useful preferred antioxidants are those included in the disclosure of U.S. Pat. No. 4,031,023, which is herein incorporated by reference.

### 3. Seal Swell Compositions

Compositions that are designed to keep seals pliable are also well known in the art. A preferred seal swell composition is isodecyl sulfolane. The seal swell agent is preferably incorporated into the composition at about 0.1-3 weight percent.

Substituted 3-alkoxysulfolanes are disclosed in U.S. Pat. No. 4,029,587, which is incorporated herein by reference.

### 4. Friction Modifiers

Friction modifiers are also well known to those skilled in the art. A useful list of friction modifiers is included in U.S. Pat. No. 4,792,410, which is incorporated herein by reference. U.S. Pat. No. 5,110,488 discloses metal salts of fatty acids and especially zinc salts and is incorporated herein by reference. Useful friction modifiers include fatty phosphites, fatty acid amides, fatty epoxides, borated fatty epoxides, fatty amines, glycerol esters, borated glycerol esters alkoxyLATED fatty amines, borated alkoxyLATED fatty amines, metal salts of fatty acids, sulfurized olefins, fatty imidazolines, molybdenum dithiocarbamates (e.g., U.S. Pat. No. 4,259,254, incorporated herein by reference), molybdate esters (e.g., U.S. Pat. Nos. 5,137,647 and 4,889,647, both incorporated herein by reference), molybdate amine with sulfur donors (e.g., U.S. Pat. No. 4,164,473 incorporated herein by reference), and mixtures thereof.

The preferred friction modifier is a borated fatty epoxide as previously mentioned as being included for its boron content. Friction modifiers are preferably included in the compositions in the amounts of 0.1-10 weight percent and may be a single friction modifier or mixtures of two or more.

Friction modifiers also include metal salts of fatty acids. Preferred cations are zinc, magnesium, calcium, and sodium and any other alkali or alkaline earth metals may be used. The salts may be overbased by including an excess of cations per equivalent of amine. The excess cations are then treated with carbon dioxide to form the carbonate.

The metal salts are prepared by reacting a suitable salt with the acid to form the salt, and where appropriate adding carbon dioxide to the reaction mixture to form the carbonate of any cation beyond that needed to form the salt. A preferred friction modifier is zinc oleate.

### 5. Extreme Pressure/Antiwear Agents

Dialkyl dithiophosphate succinates may be added to provide antiwear protection. Zinc salts are preferably added as zinc salts of phosphorodithioic acids or dithiocarbamic acid. Among the preferred compounds for use are zinc diisooctyl dithiophosphate and zinc dibenzyl dithiophosphate and amyl dithiocarbamic acid. Also included in lubricating compositions in the same weight percent range as the zinc salts to give antiwear/extreme pressure performance are dibutyl hydrogen phosphite (DBPH) and triphenyl monothiophosphate, and the thiocarbamate ester formed by reacting dibutyl amine, carbon disulfide and the methyl ester of acrylic acid. The thiocarbamate is described in U.S. Pat. No. 4,758,362 and the phosphorus-containing metal salts are described in U.S. Pat. No. 4,466,894. Both patents are incorporated herein by reference. Antimony or lead salts may also be used for extreme pressure. The preferred salts are of dithiocarbamic acid such as antimony diamyldithiocarbamate.

### 6. Viscosity Modifiers

Viscosity modifiers (VM) and dispersant viscosity modifiers (DVM) are well known. Examples of VMs and DVMs are polymethacrylates, polyacrylates, polyolefins, styrene-maleic ester copolymers, and similar polymeric substances including homopolymers, copolymers and graft copolymers. Examples of commercially available VMs, DVMs and their chemical types are listed below. The DVMs are designated by a (D) after their number. Representative viscosity modifiers that are commercially available are listed below in Table 1.

TABLE A

| Viscosity Modifier                         | Tradename                                     | Commercial Source |
|--------------------------------------------|-----------------------------------------------|-------------------|
| 1. Polyisobutylenes                        | Indopol ®                                     | Amoco             |
|                                            | Parapol ®                                     | Exxon (Paramins)  |
|                                            | Polybutylene ®                                | Chevron           |
|                                            | Hyvis ®                                       | British Petroleum |
| 2. Olefin copolymers                       | Lubrizol ® 7060, 7065, 7067                   | Lubrizol          |
|                                            | Paratone ® 8900, 8940, 8452, 8512             | Exxon (Paramins)  |
|                                            | ECA-6911                                      | Texaco            |
|                                            | TLA 347, 555(D), 6723(D)                      | Uniroyal          |
|                                            | Trilene ® CP-40, CP-60                        |                   |
| 3. Hydrogenated styrenediene copolymers    | Shellvis ® 50, 40                             | Shell             |
|                                            | LZ ® 7341, 7351, 7441                         | Lubrizol          |
| 4. Styrene, maleate copolymers             | LZ ® 3702(D), 3715, 3703(D)                   | Lubrizol          |
| 5. Polymethacrylates (PMA)                 | Acryloid ® 702, 954(D), 985(D), 1019, 1265(D) | Rohm GmbH         |
|                                            | TLA 388, 407, 5010(D), 5012(D)                | Texaco            |
|                                            | Viscoplex ® 4-950(D), 6-500(D), 1515          | Rohm GmbH         |
| 6. Olefin-graft PMA polymer                | Viscoplex ® 2-500, 2-600                      | Rohm GmbH         |
| 7. Hydrogenated polyisoprene star polymers | Shellvis ® 200, 260                           | Shell             |

Summaries of viscosity modifiers can be found in U.S. Pat. Nos. 5,157,088, 5,256,752 and 5,395,539, which are incorporated herein by reference. The VMs and/or DVMs preferably are incorporated into the fully formulated compositions at a level of up to 10% by weight.

#### 7. Pour Point Depressants (PPD)

These components are particularly useful to improve low temperature qualities of lubricating oils. A preferred pour point depressant is an alkyl naphthalene. Pour point depressants are disclosed in U.S. Pat. Nos. 4,880,553 and 4,753,745, which are incorporated herein by reference. PPDs are commonly applied to lubricating compositions to reduce viscosity measured at low temperatures and low rates of shear. The pour point depressants are preferably used in the range of 0.1-5 weight percent. Examples of tests used to access low temperature, low shear rate rheology of lubricating fluids include ASTM D97 (pour point), ASTM D2983 (Brookfield viscosity), D4684 (Mini-rotary Viscometer) and D5133 (Scanning Brookfield).

Examples of commercially available pour point depressants and their chemical types are listed in Table 2.

TABLE B

| Pour Point Depressant                        | Tradename                   | Source           |
|----------------------------------------------|-----------------------------|------------------|
| Polymethacrylates                            | Acryloid 154-70, 3003, 3007 | Rohm & Haas      |
|                                              | LZ ® 7749B, 7742, 7748      | Lubrizol         |
|                                              | TC 5301, 10314              | Texaco           |
|                                              | ECA 11039, 9153             | Exxon (Paramins) |
| Vinyl acetate/fumarate or maleate copolymers | LZ ® 662                    | Lubrizol         |
| Styrene, maleate copolymers                  |                             |                  |

#### 8. Detergents

Lubricating compositions in many cases also preferably include detergents. Detergents as used herein are preferably metal salts of organic acids. The organic acid portion of the detergent is preferably a sulphonate, carboxylate, phenate, or

#### 10

salicylate. The metal portion of the detergent is preferably an alkali or alkaline earth metal. Preferred metals are sodium, calcium, potassium and magnesium. Preferably, the detergents are overbased, meaning that there is a stoichiometric excess of metal over that needed to form the neutral metal salt.

Preferred overbased organic salts are the sulfonate salts having a substantially oleophilic character and which are formed from organic materials. Organic sulfonates are well known materials in the lubricant and detergent arts. The sulfonate compound should preferably contain on average from about 10 to about 40 carbon atoms, more preferably from about 12 to about 36 carbon atoms and most preferably from about 14 to about 32 carbon atoms on average. Similarly, the phenates, oxylates and carboxylates preferably have a substantially oleophilic character.

While the present invention allows for the carbon atoms to be either aromatic or in paraffinic configuration, it is highly preferred that alkylated aromatics be employed. While naphthalene based materials may be employed, the aromatic of choice is the benzene moiety.

The one particularly preferred component is thus an overbased monosulfonated alkylated benzene, and is preferably the monoalkylated benzene. Preferably, alkyl benzene fractions are obtained from still bottom sources and are mono- or di-alkylated compounds. It is believed, in the present invention, that the mono-alkylated aromatics are superior to the dialkylated aromatics in overall properties.

It is preferred that a mixture of mono-alkylated aromatics (benzene) be utilized to obtain the mono-alkylated salt (benzene sulfonate) in the present invention. The mixtures wherein a substantial portion of the composition contains polymers of propylene as the source of the alkyl groups assist in the solubility of the salt. The use of monofunctional (e.g., mono-sulfonated) materials avoids crosslinking of the molecules with less precipitation of the salt from the lubricant. It is preferred that the salt be overbased. The excess metal from overbasing has the effect of neutralizing acids, which may build up in the lubricant. A second advantage is that the overbased salt increases the dynamic coefficient of friction. Preferably, the excess metal will be present over that which is required to neutralize the acids at about in the ratio of up to about 30:1, preferably 5:1 to 18:1 on an equivalent basis.

The amount of the overbased salt utilized in the composition is preferably from about 0.1 to about 10 weight percent on an oil free basis. The overbased salt is usually made up in about 50% oil with a TBN range of 10-600 on an oil free basis. Borated and non-borated overbased detergents are described in U.S. Pat. Nos. 5,403,501 and 4,792,410, which are herein incorporated by reference for disclosure pertinent hereto.

#### 9. Phosphates

The lubricating compositions can also preferably include at least one phosphorus acid, phosphorus acid salt, phosphorus acid ester or derivative thereof including sulfur-containing analogs preferably in the amount of 0.002-1.0 weight percent. The phosphorus acids, salts, esters or derivatives thereof include compounds selected from phosphorus acid esters or salts thereof, phosphites, phosphorus-containing amides, phosphorus-containing carboxylic acids or esters, phosphorus containing ethers and mixtures thereof.

In one embodiment, the phosphorus acid, ester or derivative can be a phosphorus acid, phosphorus acid ester, phosphorus acid salt, or derivative thereof. The phosphorus acids include the phosphoric, phosphonic, phosphinic, and thiophosphoric acids including dithiophosphoric acid as well as the monothiophosphoric, thiophosphinic and thiophosphonic acids.

## 11

One class of compounds are adducts of O,O-dialkyl-phosphorodithioates and esters of maleic or fumaric acid. The compounds can be prepared by known methods as described in U.S. Pat. No. 3,359,203, as for example O,O-di(2-ethylhexyl) S-(1,2-dicarbobutoxyethyl)phosphorodithioate.

The dithiophosphoric acid esters of carboxylic acid esters are another class of compounds useful to the invention. Preferred are alkyl esters having 2 to 8 carbon atoms, as for example 3-[[bis(1-methylethoxy)phosphinothioyl]thio] propionic acid ethyl ester.

A third class of ashless dithiophosphates for use with the present invention includes:

(i) those of the formula



wherein R and R<sub>1</sub> are independently selected from alkyl groups having 3 to 8 carbon atoms (commercially available as VANLUBE 761 1M, from R. T. Vanderbilt Co., Inc.);

(ii) dithiophosphoric acid esters of carboxylic acid such as those commercially available as IRGALUBE® 63 from Ciba Geigy Corp.;

(iii) triphenylphosphorothionates such as those commercially available as IRGALUBE® TPPT from Ciba Geigy Corp.; and

(iv) methylene bis(dialkylthiocarbamates) wherein the alkyl group contains 4 to 8 carbon atoms. For example, methylenebis(dibutylthiocarbamate) is commercially available as VANLUBE 7723® from R. T. Vanderbilt Co., Inc.

Zinc salts are preferably added to lubricating compositions in amounts of 0.1-5 triphenylphosphorothionates wherein the phenyl group may be substituted by up to two alkyl groups. An example of this group, among others, is triphenyl-phosphorothionate available commercially as IRGALUBE® TPPT (manufactured by Ciba-Geigy Corp.).

A preferred group of phosphorus compounds are dialkylphosphoric acid mono alkyl primary amine salts, such as those described in U.S. Pat. No. 5,354,484, which is herein incorporated by reference. Eighty-five percent phosphoric acid is the preferred compound for addition to the fully formulated ATF package and is preferably included at a level of about 0.01-0.3 weight percent based on the weight of the ATF.

The amine salts of alkyl phosphates are prepared by known methods, e.g., a method disclosed in U.S. Pat. No. 4,130,494, incorporated herein by reference. A suitable mono- or diester of phosphoric acid or their mixtures is neutralized with an amine. When monoester is used, two moles of the amine will be required, while the diester will require one mole of the amine. In any case, the amount of amine required can be controlled by monitoring the neutral point of the reaction where the total acid number is essentially equal to the total base number. Alternately, a neutralizing agent such as ammonia or ethylenediamine can be added to the reaction.

The preferred phosphate esters are aliphatic esters, among others, 2-ethylhexyl, n-octyl, and hexyl mono- or diesters. The amines can be selected from primary or secondary amines. Particularly preferred are tert-alkyl amines having 10 to 24 carbon atoms. These amines are commercially available as, for example, Primene® 81 R manufactured by Rohm and Haas Co.

The sulfonic acid salts are well known in the art and are available commercially. Representative of the aromatic sul-

## 12

fonic acids that can be used in preparing the synergists of the invention are alkylated benzenesulfonic acids and alkylated naphthalenesulfonic acids having 1 to 4 alkyl groups of 8 to 20 carbons each. Particularly preferred are naphthalenesulfonates substituted by alkyl groups having 9 to 18 carbons each, as for example dinonylnaphthalenesulfonate.

## 10. Antifoamants

Antifoaming agents are well known in the art as silicone or fluorosilicone compositions. Such antifoam agents are available from Dow Corning Chemical Corporation and Union Carbide Corporation. A preferred fluorosilicone antifoam product is Dow FS-1265. Preferred silicone antifoam products are Dow Corning DC-200 and Union Carbide UC-L45. Other antifoam agents which may be included in the composition either alone or in admixture is a polyacrylate antifoamer available from Monsanto Polymer Products Co. of Nitro, West Virginia known as PC-1244. Also, a siloxane polyether copolymer antifoamer available from OSI Specialties, Inc. of Farmington Hills, Mich. may also be included. One such material is sold as SILWET-L-7220. The antifoam products are preferably included in the compositions of this invention at a level of 5 to 80 parts per million with the active ingredient being on an oil-free basis.

## 11. Rust Inhibitors

Embodiments of rust inhibitors include metal salts of alkyl naphthalenesulfonic acids.

## 30 12. Copper Corrosion Inhibitors

Embodiments of copper corrosion inhibitors that may optionally be added include thiazoles, triazoles and thiadiazoles. Example embodiments of such compounds include benzotriazole, tolyltriazole, octyltriazole, decyltriazole, dodecyltriazole, 2-mercapto-benzothiazole, 2,5-dimercapto-1,3,4-thiadiazole, 2-mercapto-5-hydrocarbonylthio-1,3,4-thiadiazoles, 2-mercapto-5-hydrocarbonyldithio-1,3,4-thiadiazoles, 2,5-bis(hydrocarbonylthio)-1,3,4-thiadiazoles, and 2,5-bis(hydrocarbonyldithio)-1,3,4-thiadiazoles.

The following examples are given for the purpose of illustrating the invention and are not intended to limit the invention. All percentages and parts are based on weight unless otherwise indicated.

## EXAMPLES

## Example 1

Water (23.5 g.), (2-ethylhexyl)tridecylamine (70.7 g., 0.226 mole) and Ergon Hygold oil (8.8 g.) are added to a 500-ml, round-bottom flask. The mixture is cooled to about 20 degrees C. and with good agitation molybdenum trioxide (16.2 g., 0.113 mole) is then added. Using a cooling bath, carbon disulfide (18.0 g., 0.237 mole) is added at such a rate that the reaction temperature does not exceed 45 degrees C. After all the carbon disulfide has been added, the mixture is agitated at 55-60 degrees C. for 30 minutes and then heated to reflux for 4.5 hours. The condenser is then set for distillation and the mixture heated to distill off most of the water. Full vacuum is then slowly applied and the temperature is maintained at 125-130 degrees C. for 2.5-3 hours. The vacuum is released and Ergon Hygold 100 oil (100 g.) is added. The product is then suction filtered at about 80 degrees C. giving a clear, dark-brown liquid (BT-521-144).

## 13

## Example 2

Water (23.5 g.), isodecyloxypropyl-isopropylamine (available from Tomah<sup>3</sup> Products as SA-14,3 ether amine) (55.3 g., ~0.23 mole) and Uninap 100 SD oil (8.8 g.) are added to a 500-ml, round-bottom flask. The mixture is cooled to about 20 degrees C. and with good agitation molybdenum trioxide (16.2 g., 0.113 mole) is then added. Using a cooling bath, carbon disulfide (18.0 g., 0.237 mole) is added at such a rate that the reaction temperature does not exceed 30 degrees C. After all the carbon disulfide has been added, the mixture is heated to reflux for about 6.5 hours. The condenser is then set for distillation and the mixture heated to distill off most of the water. Full vacuum is slowly applied and the temperature is maintained at 125-130 degrees C. for 30 minutes. The vacuum is released, more Uninap 100 SD oil (41.2 g.) is added and the product is suction filtered while still hot giving a clear, dark red-amber liquid (BT-521-167).

## Example 3

Water (23.5 g.), alkyloxypropyl-isopropylamine (alkyl=C12 to C15) (available from Tomah<sup>3</sup> Products as SA-19,3 ether amine) (80.0 g., 0.23 mole) and Uninap 100 SD oil (8.8 g.) are added to a 500-ml, round-bottom flask. The mixture is cooled to about 25 degrees C. and with good agitation molybdenum trioxide (16.2 g., 0.113 mole) is then added. Using a cooling bath, carbon disulfide (18.0 g., 0.237 mole) is added at such a rate that the reaction temperature does not exceed 40 degrees C. After all the carbon disulfide has been added, the mixture is heated to reflux for about 3.5 hours. The condenser is then set for distillation and the mixture heated to distill off most of the water. Full vacuum is slowly applied and the temperature is maintained at 125-130 degrees C. for 30 minutes. The vacuum is released and the product is suction filtered while still hot giving a clear, dark red-amber liquid (BT-521-177).

## Example 4

## Solubility Experiments

The invention also relates to lubricating compositions containing the invention molybdenum dialkyldithiocarbamates and the improved solubility of the inventive compounds in lubricating compositions. The data in Table 1 show that the inventive compounds have much better solubility than the symmetrical-amine molybdenum DTC MOLYVAN® 822 in Infineum oil at -10° C., remaining in solution for the entire 90-day test period.

TABLE 1

| LOW TEMPERATURE SOLUBILITY TEST OF INVENTIVE MOLYBDENUM DIALKYLDITHIOCARBAMATES AT 0.9 WEIGHT PERCENT IN INFINEUM ® MOTOR OIL |                                       |                        |
|-------------------------------------------------------------------------------------------------------------------------------|---------------------------------------|------------------------|
| Molybdenum Dithiocarbamate                                                                                                    | Days at -10° C. in Infineum Motor Oil | Without Haze Formation |
| MOLYVAN ® 822                                                                                                                 | 1                                     |                        |
| BT-521-144                                                                                                                    | 90*                                   |                        |
| BT-521-177                                                                                                                    | 90*                                   |                        |

\*End of test period

The data in Table 2 show that when relatively minor amounts of the invention compound, such as 15 weight percent, are mixed with molybdenum dialkyldithiocarbamates

## 14

prepared from symmetrical dialkylamines, such as MOLYVAN 822, the low temperature solubility of the symmetrical dialkylamine-based MoDTC in lubricating compositions is clearly improved. A dramatic improvement is seen at 20% or more of the invention compound.

TABLE 2

| LOW TEMPERATURE SOLUBILITY TEST OF MIXED MOLYBDENUM DIALKYLDITHIOCARBAMATES AT 0.9 WEIGHT PERCENT IN INFINEUM MOTOR OIL |                                                         |                                                                |
|-------------------------------------------------------------------------------------------------------------------------|---------------------------------------------------------|----------------------------------------------------------------|
| Weight Percent of BT-521-144 in Infineum ® Motor Oil                                                                    | Weight Percent of MOLYVAN ® 822 in Infineum ® Motor Oil | Days at -10° C. in Infineum ® Motor Oil Without Haze Formation |
| 10                                                                                                                      | 90                                                      | 1                                                              |
|                                                                                                                         | 85                                                      | 34                                                             |
|                                                                                                                         | 80                                                      | 97*                                                            |
|                                                                                                                         | 75                                                      | 97*                                                            |
|                                                                                                                         | 50                                                      | 97*                                                            |

\*End of test period

## Example 5

## SRV Friction Coefficient Data

The test procedure for frictional properties used in this example is derived from the Annual Book of ASTM Standards 2004 section 5 Petroleum Products, Lubricants, and Fossil Fuels volume 05.03 under ASTM method D 5707, "Measuring Friction and Wear Properties of Lubricating Grease using a High-Frequency, Linear-Oscillation (SRV) Test Machine". This test is described in this method under the summary of the test method as "This test method is performed on an SRV test machine using a test ball oscillated under constant load against a test disk." This testing was not modified from the original test description other than the time was reduced from 2 hours to one hour. In the "scope" of this procedure, it is stated that "this test method can also be used for determining a fluid lubricant's ability to protect against wear and coefficient of friction under similar test conditions." The test conditions are recorded on the graph below. Reducing the coefficient of friction of the base oil by additive formulation is a desired goal in lubricant formulation. Molybdenum dithiocarbamates are known to accomplish this but it is desirable to reduce this friction even further. The graph below demonstrates a further improvement of the subject invention. The compound described as 'commercial C8/C 13' is an asymmetric molybdenum dialkyl dithiocarbamate prepared according to the Tanaka patents from two symmetric amines. The results are set out graphically in FIG. 1.

The data in FIG. 1, which is summarized in Table 3, show that the invention molybdenum dithiocarbamates, BT-521-144 and BT-521-177, provide greater friction reduction than commercial C8/C 13 MoDTC and two typical lots of MOLYVAN® 822 (molybdenum dithiocarbamate sold by the R. T. Vanderbilt Company.) Thus the invention compounds improve frictional performance of molybdenum dithiocarbamates achieving lower friction coefficients over the prior art.

TABLE 3

| SRV ® FINAL FRICTION COEFFICIENTS FOR<br>MOLYBDENUM DITHIOCARBAMATES IN MOTOR OIL |                            |
|-----------------------------------------------------------------------------------|----------------------------|
| MoDTC (~440 ppm Mo)                                                               | Final Friction Coefficient |
| Commercial C8/C13                                                                 | 0.084                      |
| MOLYVAN 822 (4K092)                                                               | 0.082                      |
| MOLYVAN 822 (0G016)                                                               | 0.073                      |
| BT-521-144                                                                        | 0.068                      |
| BT-521-177                                                                        | 0.063                      |

## Example 6

## Lower Viscosity of Inventive Molybdenum Dithiocarbamates

The inventive compounds surprisingly show significantly lower viscosities than molybdenum dithiocarbamate prepared from symmetrical amine, e.g. MOLYVAN 822, at the same molybdenum concentrations, thus affording easier handling of the additive (an additional improvement over prior art). The compounds of Examples 1, 2 and 3 were each prepared at three different molybdenum concentrations by varying the amount of diluent oil added. The viscosities were determined and plotted versus the molybdenum concentration in FIG. 2, which clearly shows that the viscosity versus molybdenum content curve rises much more sharply for the C13/C13 MOLYVAN 822 than for the inventive BT-521-144, BT-521-167 and BT-521-177 compounds.

As seen in FIG. 2, the invention compounds BT-521-167 and BT-521-177 prepared from ether amines have dramatically lower viscosities than MOLYVAN 822, providing easily poured compositions with molybdenum concentrations from over 12 weight percent to almost 15 weight percent of molybdenum. The use of less diluent oil in MOLYVAN 822 will only allow about 7.5 weight percent of molybdenum before the composition becomes too viscous to be easily poured.

What is claimed is:

1. An additive for lubricating oil compositions, comprising the reaction product of: at least one asymmetrical dialkylamine of the formula R1-NH—R2

where R1 is isopropyl, and R2 is chosen from the group consisting of (a) isodecyloxypropyl and (b) alkyloxypropyl, where alkyl is one or more of C<sub>12</sub> to C<sub>15</sub>, carbon disulfide, and a molybdenum source.

2. A molybdenum dithiocarbamate composition according to the following formula, wherein R1 and R3 are isopropyl and R2 and R4 are identical and chosen from the group consisting of (a) isodecyloxypropyl and (b) alkyloxypropyl, where alkyl is one or more of C<sub>12</sub> to C<sub>15</sub>.



3. A lubricating composition, comprising a base oil and about 0.1-3% by weight of a molybdenum dithiocarbamate composition according to claim 2.

4. A lubricating composition, comprising a base oil, and combination of molybdenum dithiocarbamates being about 0.1-3% by weight of the lubricating composition, the combination comprising:

- 5 a first molybdenum dithiocarbamate according to the following formula, wherein in the first molybdenum dithiocarbamate, R1 and R3 are 2-ethylhexyl, and R2 and R4 are tridecyl, and
- 10 a second molybdenum dithiocarbamate composition according to the following formula, wherein R1, R2, R3 and R4 are the same and are selected from alkyl groups C3 to C19:



v = 1-2;  
w = 1-2;  
x + y = 2-5;  
z = 1-2

an amount of the first molybdenum dithiocarbamate being at least about 15% by weight of the total weight of the combination of molybdenum dithiocarbamates.

- 25 5. The lubricating composition of claim 4, wherein the amount of the first molybdenum dithiocarbamate is at least about 20% by weight of the total weight of the combination of molybdenum dithiocarbamates.

- 30 6. A method for preparing a molybdenum dithiocarbamate having improved viscosity and/or friction reduction, comprising reacting:

35 at least one asymmetrical dialkylamine of the formula R1-NH—R2, where R1 is isopropyl and R2 is chosen from the group consisting of (a) isodecyloxypropyl and (b) alkyloxypropyl, where alkyl is one or more of C<sub>12</sub> to C<sub>15</sub>, carbon disulfide, and a molybdenum source.

- 40 7. An additive composition comprising a combination of molybdenum dithiocarbamates, the combination comprising:

a first molybdenum dithiocarbamate according to the following formula, wherein in the first molybdenum dithiocarbamate, R1 and R3 are 2-ethylhexyl, and R2 and R4 are tridecyl,

- 45 and a second molybdenum dithiocarbamate composition according to the following formula, wherein R1, R2, R3 and R4 are the same and are selected from alkyl groups C3 to C19:



v = 1-2;  
w = 1-2;  
x + y = 2-5;  
z = 1-2

50 an amount of the first molybdenum dithiocarbamate being at least about 15% by weight of the total weight of the combination of molybdenum dithiocarbamates.

- 55 8. The additive composition of claim 7, wherein the amount of the first molybdenum dithiocarbamate is at least about 20% by weight of the total weight of the first and second molybdenum dithiocarbamates.

\* \* \* \* \*